# EUROPEAN PATENT SPECIFICATION

(11) **EP 4 299 210 B1**
(45) Date of publication and mention of the grant of the patent: **10.09.2025**
(21) Application number: 22182569.8
(22) Date of filing: 01.07.2022
(51) Int. Cl.: B22D 19/02, B22D 19/14, C21D 6/00, C22C 1/055, C22C 29/00, C22C 29/08, C22C 29/10, C21D 1/18, C22C 33/02, B22F 5/00

(54) **(W,TI)C REINFORCED MANGANESE STEEL AND METHOD OF MANUFACTURING THE SAME**
(W,TI)C VERSTÄRKTER MANGANSTAHL UND VERFAHREN ZU SEINER HERSTELLUNG
ACIER AU MANGANÈSE RENFORCÉ AU (W,TI)C ET SON PROCÉDÉ DE FABRICATION

(43) Date of publication of application: 03.01.2024
(73) Proprietor: Sandvik SRP AB, 233 81 Svedala (SE)
(72) Inventor: MELK, Latifa, 23342 Svedala (SE)
(74) Representative: Sandvik

(56) References cited:
- CN-A- 111 482 579
- US-A1- 2018 369 905

## Description

### TECHNICAL FIELD

The present invention relates to a composite material based on reinforced manganese steel and a method for making the same.

### BACKGROUND

A particular category of wear resistant steels are typically referred to as manganese steel or Hatfield steel. These materials are suitable for applications where a high toughness and a moderate abrasion resistance are required including for example use as wear parts for crushers that are subjected to strong abrasion and dynamic surface pressures due to the rock crushing action. Abrasion results when the rock material contacts the wear part and strips-off material from the wear part surface. Additionally, the surface of the wear part is subjected to significantly high surface pressures that cause wear part fatigue and breakage.

Manganese or Hadfield steel is typically characterised by having an amount of manganese, usually above 11% by weight. However, the problem with manganese steel is that it is typically too ductile for wear parts in modern crushers that are subject to extreme operating conditions, meaning the at the lifetime of the wear parts is reduced and the maintenance costs are increased. Therefore, the problem to be solved is to provide a manganese steel with enhanced wear resistance.

A known solution is to reinforce at least part of the manganese steel with particles having an increased hardness. WO20200222662 discloses a composite material, however the problem with this material is that is not provide an optimal balance between wear resistance and impact resistance and an even more significant problem is that there is poor bonding between the reinforcing particle and the manganese steel matrix and poor bonding between reinforced and non-reinforced zones, which leads reduced wear resistance and premature failure of the wear parts. Therefore, the problem to be solved is to provide a composite material that can be used for wear parts having an optimal balance between wear resistance and impact resistance, wherein there is improved bonding between the reinforcing particles and the manganese matrix and the bonding between the reinforced and non-reinforced zones in order to reduce defects and cracking that would lead to premature failure of the wear parts.

US2018/369905 A1 discloses a powder compaction used in the fabrication of casting inserts. CN111482579 A discloses a wear-resistant steel-bonded hard alloy composite hammer head and a manufacturing method thereof.

### DEFINITIONS

A "catalysis" is a metal powder or mixture of metal powders which during the reaction in the self-propagating high temperature synthesis (SHS) undergo melting and form a matrix of the composite zone. The fundamental role of catalysis is to reduce the amount of dissipated energy in the SHS process.

A "compact" is a densified powder composition.

### SUMMARY OF INVENTION

It is an objective of this invention to provide a novel and improved composite material for wear parts. The objective is achieved by providing a composite material according to independent claim 1

Advantageously, this produces a composite material that has both increased wear resistance and structural integrity. Therefore, when the material is used on areas of wear parts that are highly exposed to wear the lifetime of the parts is increased. If the average grain size of the (W,Ti)C and WC grains is too large, then the composite material will be too brittle. If the average grain size of the (W,Ti)C and WC grains in too small the wear resistance will be reduced.

Preferably, the composite material comprises between 80-98 wt% of (W,Ti)C and between 0-30% WC in each of the reinforcing zones. Preferably between 90-98 wt% of (W,Ti) C and 20-30% of WC respectively, even more preferably between 94-98 wt% and 25-30% of (W,Ti)C and WC respectively. Advantageously, this provides the optimal balance between wear resistance and impact resistance. If the wt% of (W,Ti)C and WC in each of the reinforcing zones in too high the composite material will be too brittle and more prone to failure. If the wt% of the (W,Ti)C and WC in each of the reinforcing zones is too low, then composite material will have low hardness and therefore it will not have sufficient wear resistance.

In the present invention, the composition of the manganese steel in manganese steel zone has the chemical composition by weight of: carbon: 0.5 to 2.0%; manganese: 11 to 22%; silicon: 0.2 to 1.0%; chromium: 1 to 2%; nickel: up to 0.6%; molybdenum: up to 0.5%; and a balance of Iron. Advantageously, this steel composition is characterized by the addition of micro-alloying elements such as chromium, nickel and molybdenum in good amounts which induce high yield strength and high hardness resulting in increase in wear resistance of manganese steel.

In the present invention, the Vickers hardness of the reinforcing zones is between 900-1400 HV1 and the hardness of the manganese steel zone is between 300 - 400 HV1 before work hardening. Advantageously, the increased hardness in the reinforcing zones leads to a more wear resistant material.

Preferably, the thickness of each of the interface layer is greater than 150 µm, preferably greater than 100 µm, even more preferably greater than 90 µm. Advantageously, this thickness of interface layer or thickness of contact area between manganese and composite zone is an indication of an increase in the reaction propagation rate and the amount of heat generated due to the high combustion temperature taking place at the contact between the molten Manganese steel and the insert. If the thickness is too large the heat conductivity increases in the composite zone which results in a faster heat dissipation towards the inside of the composite zone resulting in high nucleation rate of (W,Ti)C and WC particles. If the thickness is too small the heat conductivity is less which favours growth, consequently less nucleation of (W,Ti)C and WC particles.

Preferably, the interface layer is free of defects. Advantageously, the absence of any defects in the interface layer means that there is good bonding between the manganese steel zone and each of the reinforcing zones and consequently the structural integrity of the composite material is improved, meaning that the lifetime of the wear parts that the materials is used in is increased. Further, the absence of the presence of any pores is an indication that the composition has the ability to absorb the excess heat and gases from the SHS process and so therefore signifies that the synthesis reaction has been successful.

Preferably, the wettability between the (W,Ti)C and WC grains and the manganese steel in the reinforcing zone (s) is >99%, preferably >99.5%, even more preferably >99.9%. Advantageously, good wettability induces an excellent bonding between the composite zone and Manganese steel preventing defects such as pores and cracks to form and consequently the wear resistance increases. Preferably, the each of the reinforcing zones has a volume of between 30-75 cm³. Advantageously, this size provides the optimal balance between wear resistance and impact resistance.

Preferably, at least 90 %, more preferably at least 95% of the (W,Ti)C have a core-rim structure which has a rounded shape with a gradient of compositions from the centre to the outside of the particles where the core is rich in Ti and the shell is rich with W. WC grains in the reinforcing zones have an irregular prismatic shapes including triangular to rectangular shapes. Advantageously, the core-rim structure with a round shape of (W,Ti)C and the different prismatic shapes of WC will contribute to crack deflection and stop crack propagation increasing the ductility and high wear resistance of the reinforcing zone. Advantageously, the prismatic shapes of WC of will contribute to crack deflection and stop crack propagation increasing the ductility and high wear resistance of the reinforcing zone. Meanwhile, the core-rim shape will help to reduce the stress concentration under load.

Preferably, the distance between two neighbouring reinforcing zones is between 0.5-5 µm. Advantageously, this provides the optimal balance between wear resistance and impact resistance. If the reinforcing zones are spaced too far apart then the wear resistance will not be high enough. If the reinforcing zones are spaced to close together then the impact resistance will not be high enough.

Another aspect of the present invention relates to a wear part comprising the composite material as described hereinbefore or hereinafter. Advantageously, the presence of the reinforcing zones within the manganese zone will improve the wear resistance and therefore the lifetime of the wear parts which in turn increases profitability.

Another aspect of the present invention relates to a method of producing the composite material as specified in independent claim 5.

Advantageously, if this pressing pressure is used the compacts have a low density which enables the manganese steel to more easily infiltrate between the WC and TiC grains and consequently results in improved bonding between the WC and TiC grains and the manganese steel. Further it avoids the creation of defects which would lead to premature failure of the wear parts that the composite material is used in.

In the present invention, the catalysis is selected from Fe, Mn, Ni, Mo, Cr, W, Al, or a mixture thereof. Advantageously, the addition of a catalysis in a specific amount will contribute to a strong stabilization to austenite phase within the microstructure in addition to good mechanical properties and high wear resistance. The catalysis addition will also act as a grain growth inhibitor which results in a fine microstructure.

### BRIEF DECRSIPTION OF DRAWINGS

Figure 1: Shows a line drawing of the composition of the composite material.
Figure 2: Shows an SEM image taken of the reinforced zone with low magnification on the left and high magnification on the right.
Figure 3: Shows an SEM image taken of the interface layer with low magnification on the left and high magnification on the right.
Figure 4: Shows an SEM image of the composite material
Figure 5: Shows a perspective drawing of a wear part.
Figure 6: Shows defects in sample E

### DETAILED DESCRIPTION

Figure 1 shows a composite material 2 comprising at least one reinforcing zone 4 comprising tungsten carbide (W,Ti)C and tungsten carbide (WC) and a manganese steel matrix; a manganese steel zone 6 that surrounds each of the reinforcing zones 4 ; and an interface layer 8 positioned between each of the reinforcing zones 4 and the manganese steel zone 6. In each of the reinforcing zones, the (W,Ti)C and WC acts to reinforce the manganese steel matrix.

The average grain size of the (W,Ti)C particles in each of the reinforcing zone(s) (4) is between 0.2-2 µm, preferably between 1-2 The average grain size of the WC particles in each of the reinforcing zone(s) (4) is between 20-30 µm, preferably between 20-25

The average grain size of the (W,Ti)C and WC grains is measured by Scanning Electron Microscopy (SEM) analysis where several and different areas from the samples were analysed and particle sizes were measured using Image J software. Then, the average particle size was calculated.

Each interface layer 8 comprises (W,Ti)C, WC and manganese steel and can be distinguished from the reinforcing zones 4 as the shape and size of the (W,Ti)C and WC grains are different. The interface layer(s) 8 can be distinguished from the reinforcing zone(s) 4 can either: comparing the geometry and / or comparing the average grain size. If the geometry is being compared, the reinforcing zone(s) 4 comprise >90% WC grains having irregular prismatic geometry whereas the interface layer(s) 8 comprise <5% WC grains having rectangular prismatic geometry. A WC grain is considered to have rectangular prismatic geometry if the grains have 4 sharp edges. In the present invention, a (W,Ti)C is considered to have a core-rim structure with a round geometry if it has a dark colour core rich in Ti and light colour shell rich in W.

If the grain size is being compared the average WC grain size of in the interface layer(s) 8 is at least 5% less than the average WC grain size on the reinforcing zone(s) 4. Figure 2 shows a Scanning Electron microscope image using MIRA3 TESCAN equipment. A secondary electron detector (SE) with a high voltage of 15 KV and a working distance of 9 mm configuration were used. SEM image of the (W,Ti)C and WC grains in the reinforcing zone 4. Figure 3 shows an SEM image of the (W,Ti)C and WC grains in the interface layer 8. The different (W,Ti)C and WC grain geometry and size can clearly be seen when comparing these two figures.

In one embodiment the wt% of (W,TiC) in each of the reinforcing zones 4 is between 80-98 %, more preferably between 90-98 %, even more preferably between 94-98% and the wt% of WC in each of the reinforcing zones 4 is between 0-30 %, more preferably between 20-30 %, even more preferably between 25-30%.

In the present invention, the composition of the manganese steel in manganese steel zone 6 has the chemical composition by weight of: carbon: 0.5 to 2.0%; manganese: 11 to 22%; silicon: 0.2 to 1.0% ; chromium: 1 to 2%; nickel: up to 0.6%, molybdenum: up to 0.5% and a balance of Fe.

In one embodiment, the chemical composition of the manganese steel in each of the reinforcing zones 4 has the chemical composition by weight of: 1-1.5 %C, 11-14 % Mn, 0.4-0.8 % Si, 1.3-2.0 % Cr, 0.6 % Ni, 0.065 % P.

In the present invention, the hardness of the reinforcing zones 4 is between 900-1400 HV1, preferably between 1000-1400. In the present invention, the hardness of the manganese steel zone 6 is between 300 - 400 HV1 before work hardening.

Hardness is measured using Vickers hardness mapping on polished samples using a 1 kgf and a holding time of 15 seconds. A micro-hardness tester, Matsuzawa, model MXT was used. Hardness measurement profiles are performed starting from the non-reinforce zone, moving to the interface layer and then to the reinforced zone.

In one embodiment, the interface layer 6 is greater than 150 um wide, preferably greater than 100 Figure 4 shows an SEM image taken at 15.0kV, 219 magnification of the reinforced zone 4, the manganese steel zone 6 and the interface layer 8. The width of the interface layer 6 is measured from a start point 10, which is defined as being adjacent to the manganese steel zone 6 and the point at where the (W,Ti)C and WC grains are present. The end point 12 for measuring where the interface layer 8 ends, and therefore where the reinforcing zone 8 starts is considered to be where the average grain size of the WC grains has increased by 20% compared average WC grains measured at the start point 10 and / or where the percentage of WC grains having a triangular prismatic shape increases above 90%.

In one embodiment, the interface layer 8 is free of defects. Defects are considered to be cracks or pores.

In one embodiment, the wettability between the (W,Ti)C grains and the manganese steel and between the WC and the manganese steel in the reinforcing zones 4 is >99%, preferably >99.5%, more preferably >99.9%, most preferably 100%. Wettability is measured by a Scanning Electron Microscope where the contact area and the bonding between the (W,Ti)C grains or WC grains and the manganese steel have been evaluated.

In one embodiment each of the reinforcing zones 4 has a volume of between 30-75 cm³. For example, but not limited to the reinforcing zone(s) 4 could have a length of between 100-200 mm, preferably between 100-150 mm, a width of between 20-30 mm, preferably between 20-25 mm and a thickness between 15-30 mm, preferably between 15-25 mm.

In one embodiment >95%, preferably >98%, more preferably >99% of the (W,Ti)C grains in the reinforcing zones 4 have a rounded shape. Preferably, the (W,Ti)C grains are uniformly distributed in the manganese steel in the reinforcing zone(s). In one embodiment >95%, preferably >98%, more preferably >99% of the WC grains in the reinforcing zones 4 have a triangular prismatic shape. Preferably, the TiC grains are uniformly distributed in the manganese steel in the reinforcing zone(s).

In the present invention, there are a plurality of reinforcing zones 4 with its interface zone 8 and the distance between two neighbouring reinforcing zones 4 with its interface layer 8 is between 1-5 mm, preferably between 1-3 mm, more preferably between 1-2 mm.

Figure 5 shows an example of a wear part 14 comprising the composite material 2 as described hereinabove or hereinafter. For example, the wear part 2 could be, but not limited to, a cone crusher or a stationary jaw crusher or a mobile jaw crusher that is configured to crush material or other material/rock processing unit. The reinforcing zone(s) 4 are positions on the wear parts 14 in the locations that are most subjected to high wear, for example on a crushing zone 18 of a cone crusher 16.

The method for producing the composite material 2 as described hereinbefore or hereinafter comprising the steps of: a) Mixing together 65-98 wt% tungsten, preferably 80-98 wt% tungsten; 3-90 wt%, preferably 10-90 wt% Ti; 3-20 wt%, preferably 3-20% carbon and 10-20 % catalysis powders; b) compacting the mixed powders together to form at least one compact using a compacting pressure of between 400-700MPa, preferably 500-600 MPa more preferably 550-600 MPa; c) positioning and optionally fixing at least one compact into the interior of a mold; d) pouring molten casting manganese steel into the mold to surround the at least one compact to initiate a self-propagating high temperature synthesis (SHS) reaction to produce a cast; e) heat treating the cast; and then f) quenching the cast.

Preferably, the cast is treated at a temperature of between 1400-1500°C, the cast is quenched using water. In the present invention, the catalysis is selected from Fe, Co, Ni, Mo, Cr, W, Al, or a mixture thereof. Carbon could be added in the form of graphite, amorphous graphite, a carbonaceous material or mixtures thereof. The compacts could for example be held in place using me a metallic fixation system to hold them in place during casting.

### EXAMPLES

### Example 1- Samples

Sample A is a reference sample of non-reinforced manganese steel having the composition 1-1.5 %C, 11-14 % Mn, 0.4-0.8 % Si, 1.3-2.0 % Cr, 0.6 % Ni, 0.065 % P.

Samples A-I are samples of composite materials produced by mixing together powders of tungsten, titanium, carbon and a catalysis powder. The compacting the mixed powders to form compacts which were then positioned in a mold and then molten manganese steel having a composition of 1-1.5 %C, 11-14 % Mn, 0.4-0.8 % Si, 1.3-2.0 % Cr, 0.6 % Ni, 0.065 % was poured into the mold to surround the compacts which initiated a SHS reaction, the cast was then heat treated at a temperature of 1450 °C and then quenching with water. Table 1 shows a summary of the reinforced samples:
Samples A and D are reference samples, while samples B, C, F-H are inventive samples.

**Table 1: Summary of samples**

| Sample | Compacting pressure used (mPA) | Average (W,Ti)C grain size in reinforcing zone (µm) | (W,Ti)C content in reinforced zone (wt%) | Average WC grain size in reinforcing zone (µm) | WC content in reinforcing zone (wt%) | Wettability (%) |
|---|---|---|---|---|---|---|
| A | 600 | 1.88 | 98 | - | 0 | 100 |
| B (inventive) | 600 | 1.04 | 90 | 20 | 10 | 100 |
| C (inventive) | 600 | 0.95 | 94 | 25 | 30 | 100 |
| D | 600 | 0.82 | 98 | - | 0 | 100 |
| E (comparati ve) | 600 | 0.49 | 80 (pores) | - | 0 | 80 |
| F (inventive) | 600 | 0.36 | 98 | 25 | 30 | 100 |
| G (inventive) | 600 | 0.74 | 98 | 25 | 20 | 100 |
| H (inventive) | 600 | 1.27 | 98 | 25 | 30 | 100 |
| I (inventive) | 600 | 1.04 | 98 | 25 | 25 | 100 |

It can be seen if the compacting pressure is not high enough then the wettability is reduced.

### Example 2 - Hardness

Vickers hardness was measured by a micro-hardness tester, Matsuzawa, model MXT using 1 kgf and a holding time of 15 seconds. Hardness measurement profiles are performed starting from the non-reinforce zone, moving to the interface layer and then to the reinforced zone.

The hardness measurement results are shown in Table 2 below:

**Table 2: Hardness measurement**

| Sample | Hardness in manganese steel zone (HV1) | Hardness in Interface layer | Hardness in reinforced zone |
|---|---|---|---|
| A | 582±36 | 956±90 | 1267±227 |
| B (inventive) | 460±62 | 937±85 | 1111±165 |
| C (inventive) | 469±37 | 970±82 | 1067±172 |
| D | 487±32 | 920±67 | 1120±277 |
| E (comparative) | - | - | |
| F (inventive) | 552±53 | 950±81 | 1148±153 |
| G (inventive) | 450±50 | 886±19 | 1030±147 |
| H (inventive) | 472±119 | 876±86 | 1062±187 |
| I(inventive) | 621±37 | 926±30 | 1030±141 |

It can be seen that the inventive samples have an increased hardness in reinforced zones compared to the comparative samples. It was not possible to measure the hardness of E due to the large size of the pores.

### Example 3 - Defects

**Table 3: Defects**

| Sample | Defects in the reinforced zone | Defects in the interface layer |
|---|---|---|
| A | Small pores | none |
| B (inventive) | Small pores | none |
| C (inventive) | Small Pores | none |
| D | Small Pores | none |
| E (comparative) | Big pores and cracks | Big pores and cracks |
| F (inventive) | Small Pores | none |
| G (inventive) | Small Pores | none |
| H (inventive) | Small Pores | none |
| I (inventive) | Small Pores | none |

Defects were assessed by using Scanning Electron microscopy analysis where cracks and pores are identified. The inventive samples only have small pores in the reinforced zone and no defects in the interface layer.

## Claims

1. A composite material (2) comprising:
at least one reinforcing zone (4) comprising round geometry of core-rim tungsten titanium carbide (W,Ti)C,
tungsten carbide (WC) and a manganese steel matrix; wherein the core is rich in titanium and the rim is rich in tungsten;
a manganese steel zone (6) that surrounds each of the reinforcing zones (4); and
an interface layer (8) positioned between each of the reinforcing zones (4) and the manganese steel zone (6);
wherein there are a plurality of reinforcing zones (4) and the distance between two neighbouring reinforcing zones is between 1-5 mm;
wherein the hardness of the reinforcing zones (4) is between 900-1400 HV1 and the hardness of the manganese steel zone (6) is between 300 - 400 HV1 before work hardening;
wherein, the average grain size of the (W,Ti)C particles in each of the reinforcing zones (4) is between 0.2-2µm and the average grain size of the WC particles in each of the reinforcing zones (4) is between 20-30 µm wherein the average grain size of the (W,Ti)C and WC grains is measured by Scanning Electron Microscopy (SEM) analysis where several and different areas from the samples were analysed and particle sizes were measured using Image J software from which the average particle size was calculated; wherein the reinforcing zones have been
compacting with a pressure of between 400-700 MPa,
wherein the composition of the manganese steel in manganese steel zone (6) has the chemical composition by weight of: carbon: 0.5 to 2.0%; manganese: 11 to 22%; silicon: 0.2 to 1.0% ; chromium: 1 to 2%; Nickel: up to 0.6% Molybdenum: up to 0.5% and a balance of Fe.

2. The composite material (2) according to claim 1, wherein the thickness of each of the interface layer (8) is greater than 150 µm measured by Scanning Electron Microscopy (SEM) analysis.

3. The composite material (2) according to claim 1 or 2, wherein at least 90% of the WC grains in the reinforcing zones (4) have irregular prismatic shapes.

4. A wear part (14) comprising the composite material (2) according to any of claims 1-3, wherein the wear part is a cone crusher, a stationary jaw crusher or a mobile jaw crusher.

5. A method of producing the composite material (2) according to any of claims 1-4 comprising the steps of:
a) mixing together 65-98 wt% tungsten, 3-90 wt% titanium, 3-20wt% carbon and 10-20 % catalysis powders; wherein the catalysis is selected from Fe, Co, Ni, Mo, Cr, W, Al, or a mixture thereof;
b) compacting the mixed powders together to form at least one compacts (20);
c) positioning and fixing at least one compact (20) into the interior of a mold (22); wherein the distance between two neighbouring reinforcing zones is between 1-5 mm;
d) pouring molten casting manganese steel (24) into the mold (22) to surround the at least one compact (20) to initiate a self-propagating high temperature synthesis (SHS) reaction to produce a cast (26);
e) heat treating the cast (26)
f) quenching the cast (26)
wherein, in step b) the powders are compacting with a pressure of between 400-700 mPa.

## Patentansprüche

1. Verbundwerkstoff (2), umfassend:
mindestens eine Verstärkungszone (4), die eine runde Geometrie aus Kern-Rand-Wolfram-Titan-Carbid (W,Ti)C,
Wolframcarbid (WC) und einer Manganstahlmatrix umfasst; wobei der Kern reich an Titan und der Rand reich an Wolfram ist;
eine Manganstahlzone (6), die jede der Verstärkungszonen (4) umgibt; und
eine Grenzflächenschicht (8), die zwischen jeder der Verstärkungszonen (4) und der Manganstahlzone (6) positioniert ist;
wobei es eine Vielzahl von Verstärkungszonen (4) gibt und der Abstand zwischen zwei benachbarten Verstärkungszonen zwischen 1-5 mm beträgt;
wobei die Härte der Verstärkungszonen (4) zwischen 900-1400 HV1 beträgt und die Härte der Manganstahlzone (6) vor Kaltverfestigung zwischen 300-400 HV1 beträgt;
wobei die durchschnittliche Korngröße der (W,Ti)C-Partikel in jeder der Verstärkungszonen (4) zwischen 0,2-2 µm beträgt und die durchschnittliche Korngröße der WC-Partikel in jeder der Verstärkungszonen (4) zwischen 20-30 µm beträgt, wobei die durchschnittliche Korngröße der (W,Ti)C- und WC-Körner durch Rasterelektronenmikroskopie- (REM-) Analyse gemessen wird, wobei mehrere und unterschiedliche Bereiche der Proben analysiert wurden und Partikelgrößen unter Verwendung der Software Image J gemessen wurden, woraus die durchschnittliche Partikelgröße berechnet wurde; wobei die Verstärkungszonen mit einem Druck zwischen 400-700 MPa verdichtet worden sind,
wobei die Zusammensetzung des Manganstahls in der Manganstahlzone (6) die chemische Zusammensetzung nach Gewicht aufweist: Kohlenstoff: 0,5 bis 2,0 %; Mangan: 11 bis 22 %; Silizium: 0,2 bis 1,0 % ; Chrom: 1 bis 2 %; Nickel: bis zu 0,6 %; Molybdän: bis zu 0,5 % und ein Rest aus Fe.

2. Verbundwerkstoff (2) nach Anspruch 1, wobei die Dicke jeder der Grenzflächenschicht (8), durch Rasterelektronenmikroskopie- (REM-) Analyse gemessen, größer als 150 µm ist.

3. Verbundwerkstoff (2) nach Anspruch 1 oder 2, wobei mindestens 90 % der WC-Körner in den Verstärkungszonen (4) unregelmäßige prismatische Formen aufweisen.

4. Verschleißteil (14), das den Verbundwerkstoff (2) nach einem der Ansprüche 1-3 umfasst, wobei das Verschleißteil ein Kegelbrecher, ein stationärer Backenbrecher oder ein mobiler Backenbrecher ist.

5. Verfahren zum Erzeugen des Verbundwerkstoffs (2) nach einem der Ansprüche 1-4, das die folgenden Schritte umfasst:
a) Zusammenmischen von 65-98 Gew.-% Wolfram, 3-90 Gew.-% Titan, 3-20 Gew.-% Kohlenstoff und 10-20 % Katalysepulvern; wobei die Katalyse ausgewählt ist aus Fe, Co, Ni, Mo, Cr, W, Al oder einem Gemisch davon;
b) Verdichten der gemischten Pulver miteinander, um mindestens einen Pressling (20) zu bilden;
c) Positionieren und Fixieren mindestens eines Presslings (20) im Inneren einer Gussform (22); wobei der Abstand zwischen zwei benachbarten Verstärkungszonen zwischen 1-5 mm beträgt;
d) Gießen von geschmolzenem Manganstahl (24) in die Gussform (22), um den mindestens einen Pressling (20) zu umgeben, um eine sich selbst fortpflanzende Hochtemperatursynthese- (SHS-) Reaktion auszulösen, um ein Gussstück (26) zu erzeugen;
e) Wärmebehandeln des Gussstücks (26),
f) Abschrecken des Gussstücks (26),
wobei in Schritt b) die Pulver mit einem Druck zwischen 400-700 MPa verdichtet werden.

## Revendications

1. Matériau composite (2) comprenant :
au moins une zone de renforcement (4) comprenant une géométrie ronde en carbure de tungstène et de titane (W,Ti)C,
du carbure de tungstène (WC) et une matrice d'acier au manganèse ; dans lequel le centre est riche en titane et le bord est riche en tungstène ;
une zone d'acier au manganèse (6) qui entoure chacune des zones de renforcement (4) ; et
une couche d'interface (8) positionnée entre chacune des zones de renforcement (4) et la zone d'acier au manganèse (6) ;
dans lequel il y a une pluralité de zones de renforcement (4) et la distance entre deux zones de renforcement voisines est comprise entre 1 et 5 mm ;
dans lequel la dureté des zones de renforcement (4) est comprise entre 900 et 1400 HV1 et la dureté de la zone d'acier au manganèse (6) est comprise entre 300 et 400 HV1 avant écrouissage ;
dans lequel la taille de grain moyenne des particules de (W,Ti)C dans chacune des zones de renforcement (4) est comprise entre 0,2 et 2 µm et la taille de grain moyenne des particules de WC dans chacune des zones de renforcement (4) est comprise entre 20 et 30 µm, dans lequel la taille de grain moyenne de (W,Ti)C et de WC est mesurée par une analyse par microscopie électronique à balayage (MEB) dans le cadre de laquelle plusieurs zones différentes des échantillons ont été analysées et les tailles des particules ont été mesurées à l'aide du logiciel Image J à partir duquel la taille moyenne des particules a été calculée ; dans lequel les zones de renforcement ont été compactées à une pression comprise entre 400 et 700 MPa,
dans lequel la composition de l'acier au manganèse dans la zone d'acier au manganèse (6) présente la composition chimique en poids suivante : carbone : 0,5 à 2,0 % ; manganèse : 11 à 22 % ; silicium : 0,2 à 1,0 % ; chrome : 1 à 2 % ; nickel : jusqu'à 0,6 % ; molybdène : jusqu'à 0,5 % et le reste étant du Fe.

2. Matériau composite (2) selon la revendication 1, dans lequel l'épaisseur de chacune des couches d'interface (8) est supérieure à 150 µm mesurée par analyse par microscopie électronique à balayage (MEB).

3. Matériau composite (2) selon la revendication 1 ou 2, dans lequel au moins 90 % des grains de WC dans les zones de renforcement (4) présentent des formes prismatiques irrégulières.

4. Pièce d'usure (14) comprenant le matériau composite (2) selon l'une quelconque des revendications 1-3, dans laquelle la pièce d'usure est un concasseur à cône, un concasseur à mâchoires fixes ou un concasseur à mâchoires mobiles.

5. Procédé de production du matériau composite (2) selon l'une quelconque des revendications 1-4, le procédé comprenant les étapes consistant à :
a) mélanger ensemble 65 à 98 % en poids de tungstène, 3 à 90 % en poids de titane, 3 à 20 % en poids de carbone et 10 à 20 % poudres de catalyse ; dans lequel la catalyse est choisie parmi Fe, Co, Ni, Mo, Cr, W, Al ou un mélange de ceux-ci ;
b) compacter les poudres mélangées ensemble pour former au moins un compact (20) ;
c) positionner et fixer au moins un compact (20) à l'intérieur d'un moule (22) ; dans lequel la distance entre deux zones de renforcement voisines est comprise entre 1 et 5 mm ;
d) verser de l'acier au manganèse fondu (24) dans le moule (22) pour entourer l'au moins un compact (20) afin de déclencher une réaction de synthèse à haute température à autopropagation (SHS) pour produire une pièce moulée (26) ;
e) soumettre la pièce moulée (26) à un traitement thermique
f) tremper la pièce moulée (26)
dans lequel, à l'étape b), les poudres sont compactées à une pression comprise entre 400 et 700 mPa.
